

## UNITED STATES PATENT OFFICE.

FRANCIS G. OKIE, OF ST. PAUL, MINNESOTA, ASSIGNOR TO MINNESOTA MINING & MANUFACTURING COMPANY, OF ST. PAUL, MINNESOTA, A CORPORATION OF MINNESOTA.

## ABRASIVE ARTICLE.

No Drawing.

Application filed October 24, 1923. Serial No. 670,542.

To all whom it may concern:

Be it known that I, FRANCIS G. OKIE, a citizen of the United States, and a resident of St. Paul, Ramsey County, Minnesota, have invented certain new and useful Improvements in Abrasive Articles, of which the following is a specification.

My present invention relates in general to the treatment of material, preferably in sheet form, and more particularly the treatment of material for the purpose of forming or attaining composite structures, of which well known forms of abrasives such as what is commonly known as sand-paper is an example.

The present application is in part a continuation of my prior application Serial No. 428,289 filed December 4, 1920, and in part a division of my prior application Serial No. 541,248 and 541,249, filed March 4, 1922.

Although I hereinafter disclose the practice of my invention in connection with abrasives such as sand-paper, it will be understood that my invention, or certain features, thereof, have a wider field of utility.

Composite structures of the abrasive type such as sand-paper or emery cloth comprise generally (a) a base of sheet material, which may be felted as in the case of paper or woven as in the case of cloth, (b) a more or less finely comminuted resistant material having abrading properties, such as garnet or corundum, and (c) a binder generally in the form of a glue which serves to bind the abrasive to the base.

The abrasive products as produced at present have as incidents certain features among which are affinity for moisture rendering them substantially inutile in the presence of water or moisture, and cracking, with consequent exposure of the base, when bent.

The principal objects of my present invention are the provision of an abrasive article having a binder which functions more efficiently than any known to me; the provision of such an article characterized by flexibility without cracking or other un-

desirable effect; the provision of such an article being characterized by extensibility and compressibility to accommodate itself to flexion of the base; the provision of such an article having a binder by means of which the desired adhesive action between it and the base is attained not only efficiently but also with a desirable degree of acceleration, and more particularly the provision therein of a binder in which the drying action will be effective from the contact surface between it and the base outwardly; the provision of such an article having a binder in which the drying action will be effective from the outer surface inwardly; the provision therein of a binder characterized by a drying action that permits of handling the product with a minimum of delay and more particularly such handling without impairment of the surfaces of the material; the provision therein of a binder characterized by a limitation of its drying action; the provision of an improved moisture-proof material, and especially material in a sheet form, and more particularly one having means for causing a moisture proofing agent to penetrate into the material to an extent short of exudation on an adjacent surface thereof; the provision of a moisture-proof composite abrasive structure; the provision in such an article of a binder having moisture-proofing functions, and the provision generally of an improved flexible waterproof composite abrasive structure, together with such other objects and additional benefits and advantages as may hereinafter appear or be pointed out.

In the employment of my present invention for the production of sand-paper and the like (which I cite for purposes of example) I use as the base such a sheet of material (which may be paper) as will conveniently serve the employment contemplated, and as the abrasive such comminuted material (which may be crushed garnet) similarly adapted to serve the function in view.

It is desirable that the binder utilized have the functions and characteristics not

65

70

75

80

85

90

95

100

only of great mechanical strength and of great binding strength, but also that it be non-hygroscopic, permeative, moisture-resistant, easily worked, readily obtainable, inexpensive and facilely applied.

I have discovered that gums or resins of such types as are used in the manufacture

ent purposes, that manganic oxides are peculiarly useful and that borate of manganese best combines siccative energy with the desirable susceptibility to fine grinding.

Due to the otherwise relatively slow drying of the binder, difficulties are encountered in handling the structure, within a

tains shellac, red lead, litharge, manganese oxid, burnt umber, gum, linseed oil, and turpentine q. s.

In order to give the binder the desired body volumetrically considered I preferably employ a varnish consisting largely of linseed oil boiled until it reaches nearly a solid state. As far as feasible this should be as free as possible from glycerides and fatty acids.

The aforementioned gums or resins, such as gum dammar are preferably employed in the form of a varnish which is substantially three parts Batavia dammar, with two parts kettle boiled linseed oil.

While gum copal and gum kauri in certain respects make more substantial binders than gum dammar, as they will carry more oil and dry harder under certain conditions as may be useful for certain purposes, generally speaking the present relatively greater expense does not ordinarily justify their use for most purposes, which are well served by gum dammar.

Though I have hereinbefore disclosed certain forms of useful dryers having various characteristics, and likewise intensifiers, I have discovered that where it is advisable that the siccative action thereof be limited, or at least retarded, under certain conditions, or when producing material for certain purposes, that it is desirable to incorporate in the binder a non-drying oil such as castor oil or the like, for such purpose.

Sand-paper made in accordance with the disclosure of my present invention is characterized by great flexibility without any adverse effects, such as cracking of the binder or base, or loosening of one from the other; and great resistance to water, and moisture generally, and is highly resistant to deterioration in the presence of friction and moisture when used in a water-abrading operation.

The materials used by me as hereinabove described may be varied in character so as to vary the characteristics of the binder from the stand-point of adhesiveness, non-hygroscopy and flexibility. Where such variation in the use of materials is employed to produce, for instance increased adhesion between the binder and the abrasive, such increase may be attained, though possibly at a certain expense of its characteristic of flexibility.

Due, however, to this very same increased adhesiveness, one or more of the outer layers of the base may be removed as by the employment of a base which involves the use of a built up structure having a number of plies, certain of which may be removed, or by shaving off part of the thickness of the base.

By this process I am enabled to obtain sand-paper characterized by extraordinary

thinness and flexibility, in that I am able to form sand-paper and the like with a base so thin that such product could not be manufactured, if the base originally used were of the thinness ultimately desired.

In my preferred practice, I form batches which by weight and percentage contain the following ingredients:

|                             | Lbs. |
|-----------------------------|------|
| Part I Carbonate of lead    | 24   |
| Gum varnish                 | 6    |
| Part II Borate of manganese | 6    |
| Gum varnish                 | 6    |
| Part III Dryer              | 6    |
| Paste dryer                 | 6    |
| Linseed oil varnish         | 48   |
| Gum varnish                 | 42   |

This gives a composition of matter wherein metallic and resinous bases are combined in the proportions of substantially one to three; for instance, from above formula:

|                  | Lbs. |                | Lbs. |
|------------------|------|----------------|------|
| Gum varnish      | 6    | White lead     | 24   |
| Gum varnish      | 6    | Borate of man- |      |
| Gum varnish      | 42   | ganese         | 6    |
| Linseed oil var- |      | Dryer          | 6    |
| nish             | 48   |                |      |
| Dryer            | 6    |                | 36   |

108 95

The foregoing assumes that 6 parts of each of the japan and paste dryers are divided to the metallic and resinous bases.

In such preferred practice, Parts I and II are mixed and milled separately since Part I mills more readily than Part II, and are desirably then mixed with Part III and the composite batch is then milled until smooth.

Parts I and II include the gum varnish in order to attain not only a fine subdivision of the metallic substance but also to render them readily commiscible with Part III.

In the preferred practice of my invention, in forming Part I hereinabove referred to, I grind the carbonate of lead and the varnish to an exceeding fineness which may be accomplished by passing them through a fine-grinding mill three or four trips. The material grinds quickly and easily and may be conveniently mixed in the mill. One of the functions of the carbonates of lead is to hasten the oxidization of the thinner (and greasier) elements of the binder and limit their absorption by the base, e. g., paper in the case of sand-paper. It also hastens the superficial top-drying of the sand-paper or the like, rendering it among other things easier to handle before it becomes dry. Ordinary white leads, even though of apparent equal purity and of similar analyses as that herein referred to, do not function as satisfactorily for chemical reasons not yet brought to light by my ex-

70

85

100

105

110

115

125

130

perience. Gum varnish may be No. 1 gum kauri, gum copal, or gum dammar or more or less numerous similar suitable gums or resins melted in boiled or raw linseed oil, with or without the presence of dryers, such as red lead, litharge, black oxid of manganese, burnt umber, and the like. The gum varnish preferably used by me in Parts I, II and III above referred to, is substantially 5 equal parts Batavia dammar gum, and kettle boiled linseed oil. While I preferably use gum dammar, as just indicated, I have found a gum dammar varnish made from three parts Batavia dammar, melted by 10 itself under gentle heat, as is preferable though it may be used cold, and two parts of a hydrocarbon (which may be one of the petroleum series)—obviously added after the heat, if used, is discontinued. The 15 hydrocarbon referred to preferably takes the following form: Color, water white; Baumé, 48°-49°; initial boiling point, not below 275° F.; not more than 50% over at 340° F.; recovery, at least 95%; residue, 20 colorless; end point, below 475° F. As the hydrocarbon evaporates, it may be advisable to add more to the mixture in order to preserve the desired degree of fluidity. The 25 hydrocarbon dammar varnish thus formed makes a more brittle binder than the linseed oil gum dammar varnish above described. Although gum copal and gum kauri each make a more substantial binder than gum dammar, as they carry more oil 30 and dry harder, they are more expensive. Gum dammar not oxidizing to such a degree of hardness and toughness is more highly flexible, but within my experience 35 comprises as great a step towards common rosin as at present advised it appears expedient to take.

I have found that synthetic gums or resins can also be used to good advantage in making a binder for my purposes.

45 In using borate of manganese I have found that a well-known borate of manganese, readily obtainable on the open market combines best siccative energy with susceptibility to fine grinding, and to form 50 Part II referred to above it should be ground in the varnish until it may be spread on a glass without being mealy under one's finger. It should be ground until 55 experience shows that it can be ground no finer.

As will be appreciated from the foregoing discussion, the siccative energy of the borate of manganese operates from within outwardly, differing in this respect from the 60 carbonate of lead which oxidizes from without inwardly.

While I prefer to employ manganese derivatives in the form of borate of manganese, it is to be observed that although 65 black oxide of manganese contains certain

desirable siccative elements for my purposes, it does not readily lend itself to grinding in such a manner as is desired by me. At times, advantage may be taken of the characteristics of black oxide of manganese by 70 heating it in linseed oil.

Similarly, cobalt derivatives, (such as acetate of cobalt) may be employed for their siccative qualities, but I have found that due care should be employed in using such highly concentrated dryers so as to avoid any tendency toward deterioration and relative inactivity with the other dryers; failing such care such cobalt derivatives do not give such excellent effects as borate of manganese. 75

In forming Part II according to my preferred practice, I find it desirable to grind the borate of manganese by itself, ten or twelve trips if necessary, as this is relatively 85 a very hard substance to grind, and the varnish may be mixed therewith in the mill.

The form of japan-dryer preferably employed by me is a well known japan which contains about 2% (two percentum) of shell-lac, preferably the best obtainable, besides substances such as red lead ( $Pb_3O_4$ ) litharge, ( $PbO$ ) manganese oxid ( $MnO$ ) burnt 90 umber (which has a manganese and oxygen content) and gums in linseed oil and turpentine. It aids in the binding action and acts to some extent as a thinner whose turpentine content evaporates after the binder is spread on the paper and somewhat facilitates the spreading process. I have the proportion indicated in Part III as ordinarily 100 adequate but yet capable of increase with safety when larger quantities are desirable. Although to an unaccustomed observer a rosin content in the japan may, due to its rapidity of action, appear to be advantageous, 105 such a content is within my experience undesirable and to be avoided.

To form the linseed oil varnish of Part III above referred to linseed oil is boiled until nearly solid. A heavier grade than ordinary, having less glyceride and fatty acid content than is usual, although a bit more difficult to handle, has been found by me in actual practice to be slightly better. 110

In preparing the paste-dryer of Part III above referred to, I first form the initial portion of the dryer by stirring 200 pounds of litharge ( $PbO$ ) and 200 pounds of hot water (120° F.), the agitation of the water being sufficiently violent during and after the addition of the litharge to keep it from settling. After, say, two to five minutes of this sustained agitation, 45 pounds of 120 80% acetic acid is dashed into the hot-water and litharge composition without cessation of the violent stirring, which may be mechanical agitation, and which should continue until the milky white liquid that de- 125 130

velops as soon as the acid strikes the water and litharge, sets to a consistency resembling soft cottage cheese or bonny clabber and offer resistance enough to tend to slow up a 5 strong man using a paddle.

In cases where a mechanical agitator is used, it should be shut off at this stage which is ordinarily reached within a minute after the acetic acid is dashed in. It is advisable 10 to have the agitation sufficiently violent to cause suspension of all of the litharge and to dash in the acetic acid suddenly, as otherwise a quantity of uncombined litharge will be found at the bottom of the mixer, and 15 the mass, which is now basic acetate of lead, will not set stiff. This resultant mass should be undisturbed for about 15 hours and then 75 pounds kettle boiled linseed oil is added to the mass, which by this time has become 20 somewhat stiffer. The whole mass is then mixed preferably in a mechanical mixer. The mixer should be run until a large percentage of the original water may be poured off. At this time the basic acetate of lead 25 has a greater affinity for the oil than for the water. When further agitation separates out no more water, the compound should be ground. This may be done on 3 roller ink mill until no more water can be discerned, 30 and when substantially all of it can be accounted for by weighing the water that has been poured off. The strength of the acetic acid may be varied below 80% provided the proportions are changed correspondingly 35 to the strength of the acetic acid.

While the second part of the paste dryer may be formed by heating, I prefer to mix thoroughly 100 pounds of kettle boiled linseed oil, with 75 pounds of resinate of manganese (powdered form) and then grind the mixture two or three trips until fine and smooth.

I then add 225 pounds kettle boiled linseed oil to the lead compound formed in the mixer 45 as above set forth, and then quickly mix the resulting mass of the second portion with the modified first or lead compound portion which is in the mixer as just set forth.

This mixing of the two portions should 50 be done quickly because there is a nicely balanced proportion between the two, and an excess of either portion in long contact with the other portion, imperfectly mixed, causes a livering and sometimes a separation therebetween. After this mixture of the two portions has stood for substantially an hour, they should be milled one trip. This completes the paste dryer. It should flow 55 down the apron of the mill about one inch deep, (more or less, depending partly on tightness of rollers and consequent heat,) and it should be kept in stock in a consistency about like cheesy butter, but rather softer, and of a light brownish gray color. 60

65 By having the manganic derivative pre-

cipitated or combined with a more substantial gum than rosin (resinate of manganese) in the formation of this paste dryer results are attainable which from certain aspects present obvious advantages.

70

From the foregoing description it will be apparent that one of the general functions of the carbonate of lead is to serve as filler, and of the borate of manganese, as well as of the japan composition referred to, is to 75 serve as a dryer, and that the rest of my improved binder is made up of varnishes.

The gross formula of the binder considered from this aspect of the invention, therefore involves the use, generally, of four 80 parts "filler", three parts "dryer", and seventeen parts "varnish", preferably associated together in the specific manner set forth.

The binder is formed in my preferred 85 practice, by running together through the mill Parts I and II, ground finely as described, together with the items of Part III, all three parts being milled together until the whole mass is uniform and smooth. The 90 binder thus formed should be kept carefully covered preferably in contact with oiled paper to prevent the formation of surface skin through exposure.

By the term "composite" throughout the 95 specification and claims is meant a structure, mechanically or chemically produced, which is composed of a base, an abrasive, and a binder for (a) attaching the abrasive to the base; (b) rendering such bond waterproof, and (c) preventing premature destruction of the base.

Having thus described my invention and 100 illustrated its use, what I claim as new and desire to secure by Letters Patent is:

105

1. The new article of manufacture in the nature of sand paper, comprising a flexible sheet of fabric, a grit or layer of abrasive particles, and a waterproof stable adhesive bond interposed between said grit and said 110 sheet and of a nature to adequately maintain its bonding effect in substantially full measure throughout the effective abrading life of the abrasive article even under sustained application of or immersion in 115 water, but not materially affecting the flexibility of said sheet when dry.

2. The new article of manufacture in the nature of sand paper, comprising a flexible sheet of fabric, a grit or layer of 120 abrasive particles, and a waterproof stable adhesive bond including a varnish, a drier and a filler interposed between said grit and said sheet and of a nature to adequately maintain its bonding effect in substantially 125 full measure throughout the effective abrading life of the abrasive article even under sustained application of or immersion in water, but not materially affecting the flexibility of said sheet when dry.

130

3. The new article of manufacture in the nature of sand paper, comprising a flexible sheet of fabric, a grit or layer of abrasive particles, and a water proof stable adhesive bond interposed between said grit and said sheet, and of a nature to adequately maintain its bonding effect in substantially full measure throughout the effective abrading life of the abrasive article even under sustained application of or immersion in water, but not materially affecting the flexibility of said sheet when dry. 70
4. A new article of manufacture in the nature of sand paper comprising a flexible sheet of paper or material similarly susceptible to weakening by moisture, a grit or layer of abrasive particles, and a water-proof stable adhesive bond interposed between said grit and said sheet and impregnating said sheet to fully protect it against penetration by water, and of a nature to adequately maintain its bonding effect in substantially full measure throughout the effective abrading life of the abrasive article, even under sustained application of, or immersion in water, but not materially affecting the flexibility of the sheet when dry. 80
5. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation, and penetration retarding means associated therewith to limit the flux of said bond and exudation thereof onto the back of the sheet, whereby starving of the bond between the sheet and grit is obviated, and a connection which is durable is attained between the grit and sheet. 90
6. The new article of manufacture in the nature of sand paper, comprising a flexible sheet of fabric, a grit or layer of abrasive particles, and a waterproof stable adhesive bond, including an oil, interposed between said grit and said sheet and of a nature to adequately maintain its bonding effect in substantially full measure throughout the effective abrading life of the abrasive article even under sustained application of or immersion in water, but not materially affecting the flexibility of said sheet when dry. 100
7. The new article of manufacture in the nature of sand paper, comprising a flexible sheet of fabric, a grit or layer of abrasive particles, and a waterproof stable adhesive bond, including a gum, interposed between said grit and said sheet and of a nature to adequately maintain its bonding effect in substantially full measure throughout the effective abrading life of the abrasive article even under sustained application of or immersion in water, but not materially affecting the flexibility of said sheet when dry. 110
8. The new article of manufacture in the nature of sand paper, comprising a flexible sheet of fabric, a grit or layer of abrasive particles, and a water-proof stable adhesive bond including a resin interposed between said grit and said sheet of a nature to adequately maintain its bonding effect in substantially full measure throughout the effective abrading life of the abrasive article even under sustained application of or immersion in water but not materially affecting the flexibility of the article when dry. 120
9. The new article of manufacture in the nature of sand paper, comprising a flexible sheet of fabric, a grit or layer of abrasive particles, and a waterproof stable adhesive bond, including a gum varnish, interposed between said grit and said sheet and of a nature to adequately maintain its bonding effect in substantially full measure throughout the effective abrading life of the abrasive article even under sustained application of or immersion in water, but not materially affecting the flexibility of said sheet when dry. 130
10. The new article of manufacture in the nature of sand paper, comprising a flexible sheet of fabric, a grit or layer of abrasive particles, and a waterproof stable adhesive bond, including an oil and a resin interposed between said grit and said sheet and of a nature to adequately maintain its bonding effect in substantially full measure throughout the effective abrading life of the abrasive article even under sustained application of or immersion in water, but not materially affecting the flexibility of said sheet when dry. 140
11. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deterioriously affecting the flexibility of the article when dry, and means for accelerating drying of the bond. 150
12. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective 160

- abrading life of the abrasive article when employed in a water abrading operation but not deleteriously affecting the flexibility of the article when dry, and means for limiting drying of the bond. 5

13. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, means for accelerating drying of the bond, and means for limiting drying thereof. 10

14. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, means for accelerating desiccation of the bonding material from the surface which is out of contact with the air. 15

18. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, means for accelerating desiccation of the bonding material from the surface which is out of contact with the air. 20

19. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, means for accelerating desiccation of the bonding material from the surface in contact with the air, and means for accelerating desiccation thereof from the surface which is out of contact with the air. 25

15. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article, and means for limiting penetration by the bonding material, and means for accelerating drying thereof. 30

16. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, and means for accelerating desiccation of the bonding material from the surface in contact with the air. 35

20. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation, and penetration retarding means including white lead to limit the flux of said bond and exudation thereof onto the back of the sheet, whereby starving of the bond between the sheet and grit is obviated, and a connection which is durable is attained between the grit and sheet. 40

17. The new article of manufacture in the nature of sand paper, comprising a flexible sheet of paper or material similarly suscep-

sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, and means including castor oil for limiting drying of the bond.

22. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, and means including a japan dryer for accelerating desiccation of the bonding material.

23. The new article of manufacture in the nature of sand paper, comprising a flexible sheet of paper or material similarly susceptible to fluid penetration, a grit or layer

of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, and means including borate of manganese for accelerating desiccation of the bond from the surface which is out of contact with the air.

24. The new article of manufacture in the nature of sand paper, comprising a flexible sheet of paper or material similarly susceptible to fluid penetration, a grit or layer of abrasive particles, a waterproof stable adhesive bond interposed between said grit and said sheet of a nature to maintain its bonding effect throughout the effective abrading life of the abrasive article when employed in a water abrading operation but not deleteriously affecting the flexibility of the article when dry, and means including white lead for accelerating desiccation of the bond from the surface in contact with the air.

In testimony whereof I have hereunto signed my name.

FRANCIS G. OKIE.